

## UNITED STATES PATENT OFFICE

MYRON LASKIN, OF MILWAUKEE, WISCONSIN

## METHOD OF LUSTERING AND IMPROVING THE QUALITY OF LAMBSKINS AND SHEEPSKINS

No Drawing. Application filed August 19, 1929. Serial No. 387,100.

This invention relates to improvements in the method of lustering and improving the quality of lambskins and sheepskins.

Heretofore, lambskins and sheepskins, when finished for use in and on garments have had a very characteristic appearance. By means of the present invention ordinary lambskins and sheepskins may be finished so as to very materially change their appearance. The result is, that lambskins and sheepskins treated according to the present method may be attractively embodied in garments. Hence, a very important aspect of the present invention is that the treatment of lambskins and sheepskins contemplated thereby transforms said lambskins or sheepskins from their ordinary appearance to that of an appearance with greater luster, more desirable coloring effects, and silkiness.

A further object of the present invention is to provide a method of treating lambskins and sheepskins which will improve the natural life and wearing qualities of the hair or wool of the skins and which will also give to the hair or wool of the skins a very silky and full appearance and feel.

A further object of the invention is to provide a method of treating lambskins and sheepskins which will result in products which, when worn, will not fuzz out and become shaggy and which will shed water whereby the products will retain their original color and luster.

A further object of the invention is to provide a method of treating lambskins and sheepskins which will strengthen the grain of the skin nearest to the wool, whereby the workability of the leather is increased as is the life and appearance of the finished product.

A further object of the invention is to provide a method of lustering and improving the quality of lambskins and sheepskins which is very simple, is relatively inexpensive, is expeditious and practical, and is well adapted for the purposes described.

With the above and other objects in view the invention consists of the improved method of lustering and improving the quality of lambskins and sheepskins, and its

parts and steps as set forth in the claims, and all equivalents thereof.

In carrying out the improved method for the treatment of pelts, skins and hides, the dressing or tanning of the same is carried out in the usual manner for fur or wool skins and pelts. Then, the skins or pelts are prepared for dyeing by giving the same a preliminary combing and clipping, after which the skins or pelts are dyed or colored by any of the known methods now in use for this purpose or by any combination of the same.

After the dyeing step, the skins or pelts are treated with an oil or fat emulsion, which treatment is carried out by an immersion method, using either a drum, paddle vat, or a tub. This step serves to give oil to the leather, as well as to the wool or fur, which will enhance the feel and appearance of the finished product. This treatment also strengthens the grain nearest the wool or fur and thus increases the workability of the same as well as the life and appearance of the finished product. For said oil treatment

any of the following oils may be used: neat's-foot, castor, olive, and so forth, and said oils may be used with or without the addition of unsaponifiable oils such as mineral oils, sperm oil, and wool grease. In carrying out this step it has been found practical and successful to use in a vat one gallon of sulphonated neat's-foot oil (for example) with one hundred gallons of water. If an unemulsified oil is used it may be emulsified by some emulsifying agent such as gum, albumin, soap, alkali, or a soluble oil. So far as is known, the above method of applying oils to skins or pelts by direct immersion is new and is far more effective, as well as cheaper, than the introduction of oil by merely swabbing the leather side. Furthermore, applying the oil by direct immersion serves to enrich the wool fiber with oil.

The next step in the treatment of the pelts or skins is for the purpose of removing therefrom excess water and this is accomplished by pressing the skins or pelts or by centrifugating the same. After the excess water has been removed the skins are dried and then they are dampened and milled in sawdust

containing an emulsion mixture of oil and water to prevent bleeding of the oil used in the before-described immersion step. For the milling step a satisfactory proportion of ingredients is as follows: 300 pounds of sawdust; 7 gallons of water, and 1 gallon of sulphonated neat's-foot oil, olive oil, or a like oil. Following the milling the skins or pelts are combed, beaten and clipped, after which they are stretched and dried and then buffed and are ready for the finishing operations.

To further enhance the luster, feel and appearance of certain duller skins or pelts it is desirable to give the same a light coating of oil applied to the wool either by spray or by hand. For this purpose white paraffine oil has been found to be highly satisfactory. Following the application of the light coating of oil, the skins or pelts are "electrified" by being gone over by a hot iron and comb and are next beaten and clipped by machine. To increase the permanence and wearing qualities of what is put into and given to the pelts and skins by the oiling, "electrifying," beating and clipping operations, these operations are repeated.

From the foregoing description it will be seen that the improved method of treating lambskins and sheepskins results in products of superior quality and appearance, and the wool of said products have an unusual luster and the life of the same is increased.

What is claimed as the invention is:

1. The method of treating lambskins and sheepskins which consists of tanning the same, then combing and clipping the wool sides thereof, dyeing the skins, and then introducing directly onto and into the skins an oil emulsion.

40 2. The method of treating skins which consists of immersing said skins directly in a fat emulsion, and then removing the skins after they have become saturated.

3. The method of treating lambskins and sheepskins which consists of directly immersing said skins in a vat containing oil and water in the proportion of one part of oil to one hundred parts of water, and then removing the skins after they have become saturated.

4. The method of treating lambskins or sheepskins which consists of tanning the same, then combing and clipping the wool sides thereof, dyeing the skins, then directly immersing said skins in a vat containing an emulsion of oil and water in the proportion of about one part of oil to one hundred parts of water, and then removing the skins from the vat after the emulsion therein has saturated the skins.

5. The method of treating tanned and dyed lambskins which consists in immersing the same in a fatty emulsion for a period sufficient to saturate the skins, then drying and pressing the skins, and then dampening the

skins and milling the same in sawdust mixed with a fatty emulsion.

6. The method of treating tanned and dyed lambskins and sheepskins which consists in immersing the same in a fatty emulsion, removing the skins after they have absorbed some of the fatty material, then drying and pressing the skins, and then dampening the skins and milling the same in sawdust mixed with a fatty emulsion in the proportion of three hundred pounds of sawdust to seven gallons of water and one gallon of oil.

7. The method of treating tanned and dyed lambskins and sheepskins which consists in immersing the same in a fatty emulsion, removing the skins from the emulsion after a relatively short time interval, then drying the same, then milling the skins in sawdust mixed with a fatty emulsion, and finally applying a hot iron to the wool sides of the skins.

8. The method of treating tanned and dyed lambskins and sheepskins which consists in immersing the same in a fatty emulsion sufficiently long for the skins to become saturated, then withdrawing and drying the same, then milling the skins in sawdust mixed with a fatty emulsion, then combing, beating, clipping, stretching and drying the skins, and finally applying a hot iron to the wool sides thereof.

9. The method of treating lambskins and sheepskins which consists of first tanning and dyeing the same, then giving the wool sides a preliminary combing and clipping, directly immersing the skins in a vat containing an emulsion of oil and water in the proportions of about one part of oil to one hundred parts of water, removing the skins from the vat after they have become saturated, then drying and pressing the skins, next dampening the skins and milling the same in sawdust mixed with a fatty emulsion in the proportions of about three hundred pounds of sawdust to seven gallons of water and one gallon of oil, then combing, beating, clipping, stretching, drying and buffing the skins, then lustering the wool sides of the same by applying a light coating of oil, and finally ironing and combing the skins, after which the pelts are beaten and clipped.

10. The method of treating sheepskins and lambskins, which consists of first tanning and dyeing the same, then giving the wool sides a preliminary combing and clipping, then combing, beating, clipping, stretching, dyeing and buffing the skins, and finally applying a hot iron to the skins, after which the skins are beaten and clipped.

In testimony whereof, I affix my signature.

MYRON LASKIN.